



US006165061A

**United States Patent** [19]**Fujii et al.****Patent Number:** **6,165,061****Date of Patent:** **Dec. 26, 2000**

[54] **ABRASIVE TAPE, PROCESS FOR PRODUCING IT, AND COATING AGENT FOR ABRASIVE TAPE**

[75] Inventors: **Kazuhito Fujii; Masahisa Yamaguchi; Takaki Miyachi; Kojiro Okawa; Yasuki Suзуura**, all of Tokyo-To, Japan

[73] Assignee: **Dai Nippon Printing Co., Japan**

[21] Appl. No.: **09/276,088**

[22] Filed: **Jan. 7, 1999**

**Related U.S. Application Data**

[63] Continuation of application No. 08/627,174, Apr. 3, 1996, abandoned.

**Foreign Application Priority Data**

Apr. 10, 1995 [JP] Japan ..... 7-109088  
Jan. 16, 1996 [JP] Japan ..... 8-05212

[51] **Int. Cl.**<sup>7</sup> ..... **B24D 3/02; B24D 11/00**

[52] **U.S. Cl.** ..... **451/533; 51/308; 451/539**

[58] **Field of Search** ..... 51/293, 294, 297, 51/300, 307, 308, 309; 451/526, 533, 534, 539

**[56] References Cited****U.S. PATENT DOCUMENTS**

|           |         |                   |
|-----------|---------|-------------------|
| 4,169,337 | 10/1979 | Payne .           |
| 4,818,806 | 4/1989  | Kunimune et al. . |
| 5,089,330 | 2/1992  | Sato et al. .     |
| 5,109,638 | 5/1992  | Kime, Jr. .       |
| 5,162,426 | 11/1992 | Hazan et al. .    |
| 5,213,589 | 5/1993  | Ronning et al. .  |
| 5,296,582 | 3/1994  | Fujita et al. .   |
| 5,314,514 | 5/1994  | Sato .            |
| 5,456,734 | 10/1995 | Ryoke et al. .    |
| 5,611,826 | 3/1997  | Ryoke et al. .    |
| 5,633,068 | 5/1997  | Ryoke et al. .    |
| 5,686,550 | 11/1997 | Noto et al. .     |
| 5,709,922 | 1/1998  | Ono et al. .      |

**FOREIGN PATENT DOCUMENTS**

WO 96/01721 1/1996 WIPO .

**OTHER PUBLICATIONS**

Patent Abstracts of Japan, vol. 12, No. 459 (M-770), Dec. 2, 1988 & JP 63 185577 A (Fuji Photo Film Co. Ltd.) Aug. 1, 1988 \*abstract\*.

Patent Abstracts of Japan, vol. 17, No. 622 (C-1130), Nov. 17, 1993 & JP 05 192639 A (Koransha Co. Ltd.), Aug. 3, 1993 \*abstract\* & Database WPI Section Ch. Week 9335, Derwent Publications Ltd., London, GB; Class LP, AN 93-277624 (35) & JP 05 192 639A (Koransha K.K.), Aug. 3, 1993 \*abstract\*.

Patent Abstracts of Japan, vol. 13, No. 327 (M-854), Jul 24, 1989 & JP 01 109083 A (Tokyo Jiki Insatsu K.K.), Apr. 26, 1989, \*abstract\* & Database WPI Section CH. Week 8923, Derwent Publications Ltd., London, GB; Class ALP, AN 89-168690 (23) & JP 01 109 083 A (Tokyo Jiki Insatsu K.K.), Apr. 26, 1989, \*abstract\*.

Patent Abstracts of Japan, vol. 12, No. 83 (M-677), Mar. 16, 1989 & JP 62 224581 A (Fuji Photo Film Co. Ltd.), Oct. 2, 1987, \*abstract\* & Database WPI, Section Ch. Week 8745, Derwent Publications Ltd., London, GB; Class ALP, AN 87-317124 (45) & JP 62 224 581 A (Fuji Photo Film Co. Ltd.), Oct. 2, 1987, \*abstract\*.

Patent Abstracts of Japan, vol. 14, No. 119 (M-0945), Mar. 6, 1990 & JP 01 316172 A (Dai Nippon Printing Co. Ltd.), Dec. 21, 1989, \*abstract\* & Database WPI, Section Ch, Week 9006, Derwent Publications Ltd., London, GB; & JP 01 316 172 A (Dai Nippon Printing Co., Ltd.), Dec. 21, 1989, \*abstract\*.

*Primary Examiner*—Timothy V. Eley

*Attorney, Agent, or Firm*—Parkhurst & Wendel, LLP

**[57] ABSTRACT**

Provided are an abrasive tape suitable for finishing of surfaces or the like of precision components such as optical connector ferrules and semiconductor wafers, and a process for producing it. A coating agent in which abrasive particles having an average particle size in the range of 1 to 200  $\mu$ m are dispersed in a binder resin solution. The coating agent is applied, with intervention of a primer layer if necessary, onto a base for abrasive tape to form an abrasive layer, thus obtaining an abrasive tape.

**7 Claims, 2 Drawing Sheets**





FIG. 1



FIG. 2



FIG. 3

## 1

**ABRASIVE TAPE, PROCESS FOR  
PRODUCING IT, AND COATING AGENT  
FOR ABRASIVE TAPE**

This is a Continuation of application Ser. No. 08/627,174 filed Apr. 3, 1996 now abandoned.

**BACKGROUND OF THE INVENTION**

1. Field of the Invention

The present invention relates to an abrasive tape suitably applicable to finishing of surfaces, end faces, and so on of precision components such as optical connector ferrules, semiconductor wafers, metals, ceramics, color filters (for liquid crystal display or the like), plasma displays, optical lenses, substrates of magnetic disk or optical disk, magnetic heads, and optical reading heads, a process for producing it, and a coating agent for abrasive tape.

2. Related Background Art

The precision in grinding for finishing affects the quality of the precision components such as the optical connector ferrules and the semiconductor wafers, and grinding called mechanical polishing has been and is employed for finish grinding.

The mechanical polishing is carried out as follows. First, abrasive particles having particle diameters of 5 to 300  $\mu$  are suspended in an alkaline solution such as caustic soda, ammonia, or ethanolamine to prepare an abrasive solution consisting of a colloidal solution of pH 9 to 12. While this abrasive solution is next supplied onto an abrasive cloth comprised of a resin sheet, for example a polyurethane sheet, a precision component such as the optical connector ferrule or the semiconductor wafer is ground on the abrasive cloth.

The above mechanical polishing using the abrasive solution and abrasive cloth has the following problems.

Changes will occur in the concentration of abrasive particles in the abrasive solution during grinding and in the particle size distribution of abrasive particles due to cohesion of abrasive particles, which could result in forming grinding scars or grinding spots on the ground body such as the optical connector ferrule or the semiconductor wafer. The mechanical polishing needs a process for washing the abrasive particles adhering to the surface of the ground body such as the optical connector ferrule or the semiconductor wafer away after completion of grinding, which makes the polishing step complex.

Against it, there is an idea to produce an abrasive tape obtained by applying a coating agent in which the abrasive particles are dispersed in a binder resin solution, onto a base for abrasive tape made of a plastic film and drying it to form an abrasive layer. The optical connector ferrules and semiconductor wafers, etc. are ground on this abrasive tape, but it cannot be used as an abrasive tape for finishing, because it is difficult in producing the abrasive tape to keep the abrasive particles of the particle diameters of 1 or less  $\mu$  uniformly dispersed in the binder resin solution.

Namely, the high precision grinding for finishing is grinding with fine abrasive particles, but with a decrease in the particle diameters of abrasive particles it becomes difficult to uniformly disperse the fine abrasive particles in the binder because cohesion becomes likely to occur because of an increase in surface energy.

When the abrasive layer is formed from the coating agent containing the abrasive particles in a cohesive state, coarse particles of 5 to 10 $\mu$  are produced in the abrasive layer, which unavoidably form grinding scars on the surface of the ground body.

## 2

**SUMMARY OF THE INVENTION**

The present invention has been accomplished under the above circumstances, and an object of the invention is to provide an abrasive tape in which the abrasive particles include no coarse particles in the abrasive layer but include only fine abrasive particles, which can realize precise mirror finishing of precision components such as the end faces of optical connector ferrules and the surfaces of semiconductor wafers, a process for producing it, and a coating agent for abrasive tape.

A first aspect of the present invention is an abrasive tape comprising: a base for abrasive tape; and an abrasive layer formed on the base; wherein the abrasive layer is formed from a coating agent in which abrasive particles of an average particle size in the range of 10 to 100  $\mu$  are dispersed in a binder resin solution, with respect to a base for abrasive tape.

A second aspect of the present invention is a process for producing an abrasive tape, comprising the steps of dispersing abrasive particles of an average particle size in the range of 10 to 100  $\mu$  in a binder resin solution, producing aggregates of the abrasive particles in the binder resin solution to obtain a coating agent containing the abrasive particles of particle diameters 50 to 800  $\mu$ , and applying the coating agent onto a base for abrasive tape.

A third aspect of the present invention is an abrasive tape comprising: a base for abrasive tape; and an abrasive layer formed on the base; wherein the abrasive layer has abrasive particles of an average particle size in the range of 1 to 200  $\mu$  and a binder for binding the abrasive particles.

A fourth aspect of the present invention is a coating agent for production of an abrasive tape, comprising an abrasive particle solution containing abrasive particles of an average particle size in the range of 1 to 200  $\mu$  and a solvent for abrasive particles, and a binder resin solution containing a binder and a binder solvent.

A fifth aspect of the present invention is a process for producing an abrasive tape, comprising: the steps of preparing a base for abrasive tape; mixing an abrasive particle solution containing abrasive particles of an average particle size in the range of 1 to 200  $\mu$  and a solvent for abrasive particles, with a binder resin solution containing a binder and a binder solvent to produce a coating agent; applying the coating agent onto the base for abrasive tape; and drying the coating agent thus applied.

According to the first aspect of the present invention, the abrasive layer is formed by applying the coating agent in which the abrasive particles of the average particle size in the range of 10 to 100  $\mu$  are dispersed in the binder resin solution, onto the base for abrasive tape, whereby the abrasive particles in the abrasive layer can be fine particles having small and close particle diameters.

According to the second aspect of the present invention, the abrasive particles of the average particle size in the range of 10 to 100  $\mu$  are dispersed in the binder resin solution, thereafter aggregates of the abrasive particles are produced in the binder resin to obtain the coating agent containing the abrasive particles of particle diameters 50 to 800  $\mu$ , and then the coating agent is applied onto the base for abrasive tape, whereby the abrasive tape can be obtained with fine particles having small and close particle diameters of the abrasive particles in the abrasive layer.

According to the third aspect of the present invention, the average particle size of the abrasive particles in the abrasive layer formed on the base for abrasive tape can be kept between 1 and 200  $\mu$ .

According to the fourth aspect of the present invention, the coating agent containing the abrasive of the average particle size in the range of 1 to 200  $\mu$  can be readily obtained.

According to the fifth aspect of the present invention, the abrasive tape having the abrasive layer containing the abrasive of the average particle size in the range of 1 to 200  $\mu$  can be produced.

#### BRIEF DESCRIPTION OF THE DRAWINGS

FIG. 1 is a drawing to show a grinding step using the abrasive tape according to the present invention;

FIG. 2 is a drawing to show a layer structure of the abrasive tape; and

FIG. 3 is a drawing to show a grinding operation of an optical connector ferrule.

#### DESCRIPTION OF THE PREFERRED EMBODIMENTS

##### First Embodied Form

Embodied forms of the present invention will be explained by reference to the drawings. FIG. 1 and FIG. 2 are drawings to show the first embodied form of the present invention.

FIG. 1 shows a precision component in a flat plate form, for example a semiconductor wafer 1. Such a semiconductor wafer 1 is subjected to finish grinding by the abrasive tape 10 (see FIG. 1). The flat-plate semiconductor wafer 1 is made of silicon.

As shown in FIG. 1, the abrasive tape 10 is placed through an elastic body 15 of an elastomer on a rotating metal plate 16.

The abrasive tape 10 is next explained referring to FIG. 2. As shown in FIG. 2, the abrasive tape 10 is composed of a base 11 for abrasive tape made of a polyester film or the like, a primer layer 12 mainly containing an epoxy resin, an acrylic resin, or a polyester resin, formed on the base 11 for abrasive tape, and an abrasive layer 13 formed on the primer layer 12. In this case, the abrasive tape 10 may be formed in a sheet form or in a band form. The primer layer 12 is not always essential, and is given taking adhesion between the base 11 and the abrasive layer 13 into consideration, depending upon materials forming them.

The abrasive layer 13 is formed by applying a coating agent in which the abrasive particles of an average particle size in the range of 10 to 100  $\mu$  (nanometer nm) are dispersed in a binder resin solution, onto the primer layer 12 on the base 11 for abrasive tape. The primer layer 12 is not always essential.

When the abrasive layer is formed by applying the coating agent in which the abrasive particles of the average particle size in the range of 10 to 100  $\mu$  (millimicron) are dispersed in the binder resin solution, onto the base 11 for abrasive tape, the particle diameters of the abrasive particles in the abrasive layer 13 become between 50 and 800  $\mu$ .

In producing the abrasive tape 10, the abrasive particles of the average particle size in the range of 10 to 100  $\mu$  are dispersed in the binder resin solution, and thereafter aggregates of the abrasive particles are formed in the dispersion to prepare the coating agent containing the abrasive particles of particle diameters between 50 and 800  $\mu$ . Next, the coating agent is applied to the base for abrasive tape to produce the abrasive tape 10.

In the abrasive tape 10 of the present invention in the above structure and the process for producing it, the abrasive particles of the average particle size in the range of 10 to 100  $\mu$  may be a silica sol or an alumina sol.

When silica or alumina of particle diameters of 1 or less  $\mu$  is dispersed in the binder resin solution, coarse particles of 5 to 10  $\mu$  are likely to be made. If the abrasive tape 10 should have the abrasive layer 13 formed utilizing such silica or alumina, grinding scars would be formed on the ground body because of the coarse particles in the abrasive layer 13.

In contrast with it, when silica or alumina of the average particle size in the range of 10 to 100  $\mu$  is dispersed in the binder resin solution, the above coarse particles of 5 to 10  $\mu$  are not formed, and thus, the abrasive tape having the abrasive layer 13 formed from such a coating agent is an abrasive tape suitable for finishing of the end face of optical connector ferrule and the surface of semiconductor wafer 1.

In order to obtain the abrasive layer 13 suitable for finishing and having high abrasiveness, the particle diameters of the abrasive particles in the abrasive layer 13 need to be between 50 and 800  $\mu$ .

The abrasive layer 13, in which the particle diameters of the abrasive particles are in the range of 50 to 800  $\mu$ , can be obtained by combination of the following conditions (1) and (2).

(1) To use nearly spherical silica or alumina particles having the average particle size in the range of 10 to 100  $\mu$  as the abrasive particles in preparing the coating agent for forming the abrasive layer 13.

(2) To grow aggregates of the abrasive particles in the step of obtaining the coating agent by dispersing the abrasive particles in the binder resin solution or in the step of applying the coating agent in which the abrasive particles are dispersed in the binder resin solution, onto the base for abrasive tape, thereby obtaining the abrasive particles of particle diameters 50 to 800  $\mu$ .

The particle diameters of silica particles dispersed in the binder resin solution can be adjusted between 50 and 800  $\mu$  in such a manner that the dispersion in which the silica particles are dispersed in the binder resin solution is adjusted at pH of 7 to 9, the dispersion is slowly stirred for several hours to form aggregates of silica particles, and thereafter the resultant is filtered by a filter of 0.8  $\mu$  to remove coarse particles.

If the binder resin solution has a silicone resin or a silicone based resin having the framework of Si atoms, the particle size distribution of the silica particles in the abrasive layer becomes narrower, thereby forming a more preferable abrasive layer 13.

Presumably, the reason is that, because the silicone resin or the silicone based resin as the binder resin solution has high affinity to the silica particles, the silica particles also come to cohere when the binder resin becomes solidified in the application and drying steps of the coating agent for forming the abrasive layer.

The base 11 for abrasive tape above which the abrasive layer 13 is formed in the above structure may be synthetic paper or a plastic film having excellent properties in mechanical strength, dimensional stability, heat resistance, etc., as described above, preferably about 20 to 100  $\mu$  thick, for example selected from polyethylene terephthalate, oriented polypropylene, polycarbonate, acetyl cellulose diester, acetyl cellulose triester, oriented polyethylene, and polybutylene terephthalate.

In this embodied form, the abrasive layer 13 is formed by applying the coating agent in which the abrasive particles of the average particle size in the range of 10 to 100  $\mu$  are dispersed in the binder resin solution, to the base 11 for abrasive tape, with intervention of the primer layer if necessary, whereby the coarse abrasive particles of 5 to 10  $\mu$  are not formed in the abrasive layer 13. Using the abrasive

tape **10** obtained in this manner, finishing of the end face of optical connector ferrule or the surface of semiconductor wafer **1** can be carried out without forming grinding scars or grinding spots on the surface of the ground body.

The abrasive tape **10** having the abrasive layer **13** in which the particle diameters of abrasive particles are between 50 and 800  $\mu$  is suitable for the abrasive tape **10** for finishing the end face of optical connector ferrule and the surface of semiconductor wafer **1**, etc., which is an abrasive tape **10** with high grinding performance.

#### Second Embodied Form

The second embodied form of the present invention is next explained. The second embodied form is substantially the same as the first embodied form except for the structure of the abrasive layer **13** in the abrasive tape **10**. Namely, the abrasive tape **10** is composed of the base **11** for abrasive tape made of a polyester film or the like, the primer layer **12** mainly containing an epoxy resin, an acrylic resin, or a polyester resin and formed on the base **11** for abrasive tape, and the abrasive layer **13** formed on the primer layer **12**. The above primer layer **12** is not always essential, and is provided taking account of adhesion or the like of the base **11** and the abrasive layer **13**, depending upon the materials forming the abrasive tape base **10**, the abrasive layer **13**, etc.

In the above structure the abrasive layer **13** has the abrasive particles of the average particle size in the range of 1 to 200  $\mu$  (nanometer nm), for example colloidal silica particles, and the binder for binding the silica particles, for example an organic-inorganic composite polymer resin. In this case the organic-inorganic composite polymer resin is a polymer compound having the siloxane bonding in the structure.

In the abrasive layer **13** the colloidal silica particles are dispersed without cohesion as maintaining the average particle size in the range of 1 to 200  $\mu$ , and the total ray transmittance of the abrasive layer **13** is between 60 and 95% and the haze thereof is between 1 and 70%.

The arithmetical mean deviation (Ra) of the surface of the abrasive layer **13** is between 0.005 and 0.5 $\mu$ , and in most cases Ra is within the range of 0.007 to 0.2 $\mu$ .

Materials for the respective components will be described in more detail.

#### (1) Concerning the Binder in the Abrasive Layer

In the present invention, the binder may be a monomer, a prepolymer or oligomer, or a polymer having the siloxane bonding (Si—O bonding) in its structure, for example selected from a polysiloxane, derivatives thereof, modifications thereof, or blends thereof, and further a monomer, a prepolymer or oligomer thereof, etc.

Specifically, the binder may be, for example, not only the monomer, the prepolymer or oligomer, or the polymer, forming the polysiloxane, but also a blend, a reaction modification, or the like of the monomer, the prepolymer or oligomer, or the polymer forming the polysiloxane, for example mixed with a monomer, a prepolymer or oligomer, or a polymer forming one of polyethylene based resins, polyvinyl chloride based resins, polyvinyl acetate based resins, polyacrylic based or polymethacrylic based resins, polyvinyl alcohol based resins, ethylene copolymers, polyvinyl acetal based resins, rubber based resins, polyester based resins, polyamide based resins, phenol based resins, aminoplast based resins, epoxy based resins, polyurethane based resins, silicone based resins, cellulose based resins, and other resins.

Particularly, in the present invention, it is preferred to use a blend or a reaction modification in which the prepolymer or oligomer or the polymer of polysiloxane is mixed with a prepolymer or oligomer or a polymer of one selected from

the polyethylene based resins, polyvinyl chloride based resins, polyvinyl acetate based resins, polyacrylic based resins, polyurethane based resins, and polyester based resins.

Explaining in further detail, in the present invention a desired material for the binder may be selected from organic-inorganic composite polymers having organic main chains and inorganic side chains of siloxane bonding, obtained by binding the main chains of a prepolymer or oligomer or a polymer of one of the polyethylene based resins, polyvinyl chloride based resins, polyvinyl acetate based resins, polyacrylic based resins, polyurethane based resins, and polyester based resins with the side chains of the prepolymer or oligomer or the polymer of polysiloxane for example by graft polymerization or the like; prepolymers or oligomers thereof, etc.

Use of the organic-inorganic composite polymer as described above presents the advantage that the abrasive particles can maintain the state of primary particles without cohesion in the coating agent or in the abrasive layer, whereby the abrasive tape suitable for fine grinding can be produced.

It is not clearly known why the abrasive particles can maintain the state of primary particles as described above in the present invention, but it is presumed that, as detailed later, if the resin used as the binder has the siloxane bonding (Si—O bonding) and, for example, when the colloidal silica particles are used as the abrasive particles, the binder and silica particles will have functional groups of Si atoms common to each other, and have affinity to each other, whereby the abrasive particles can maintain the state of primary particles even in the state of a composition as the coating agent or in the state of the abrasive layer in a coating film form, enabling to produce the abrasive tape realizing very good grinding finishing.

#### (2) Concerning the Primer Layer

In the present invention, the primer layer may be formed by coating or printing of a composition with a vehicle mainly containing one or more of a monomer, a prepolymer or oligomer, or a polymer forming a resin, for example selected from polyvinyl chloride based resins, polyvinyl acetate based resins, polyacrylic based or polymethacrylic based resins, polyvinyl alcohol based resins, ethylene copolymers, polyvinyl acetal based resins, rubber based resins, polyester based resins, polyamide based resins, phenol based resins, aminoplast based resins, epoxy based resins, polyurethane based resins, silicone based resins, cellulose based resins, and other resins.

Further, a curing agent such as isocyanate may be added in order to enhance adhesion.

#### (3) Concerning the Abrasive Particles in the Abrasive Layer

In the present invention, the abrasive particles may be of an inorganic compound, for example selected from alumina (aluminum oxide), titanium oxide, zirconia (zirconium oxide), lithium silicate, diamond, silicon nitride, silicon carbide, iron oxide, chromium oxide, silica (silicon dioxide), and antimony oxide.

Since the abrasive sheet suitable for fine grinding is produced in the present invention, the above abrasive particles are preferably those having the particle diameters in the range of about 1 to 300  $\mu$ , more preferably in the range of about 1 to 200  $\mu$ , and in the state of primary particles.

Particularly, in the present invention, use of silica (silicon dioxide) is most preferred as abrasive particles, considering the affinity and compatibility with the binder.

In the present invention, when the abrasive particles are, for example, of the particle diameters of 5 to 50  $\mu$  and

when the formulation rate (% by weight) of the abrasive particles and the binder is in the range of 90:10 to 60:40, the abrasive sheet obtained is a relatively transparent abrasive sheet having the total ray transmittance in the range of 90 to 95% and the haze in the range of 2 to 15%, and the abrasive sheet has an aptitude for finish grinding of the surface of precision component such as the optical connector ferrule.

When the abrasive particles are, for example, of the particle diameters in the range of 50 to 200  $\mu\text{m}$  and when the formulation rate (% by weight) of the abrasive particles and the binder is in the range of 90:10 to 30:70, the abrasive sheet obtained becomes a relatively cloudy white or semi-transparent abrasive tape and has an aptitude for finish grinding of the surface of precision component such as the optical connector ferrule, similarly as described above.

The above phenomenon is particularly outstanding when silica particles are used as the abrasive particles.

In the present invention, if the abrasive particles become less than the binder in the formulation rate of the abrasive particles and the binder, the surface finish grinding aptitude of the abrasive tape obtained tends to be somewhat degraded.

For example, when the particle diameters are of 5 to 50  $\mu\text{m}$  and when an amount of the binder is increased to be more than that of the abrasive particles in the formulation rate (% by weight) of the abrasive particles and binder, the surface finish grinding aptitude of the abrasive tape obtained shows a tendency to be considerably lowered.

The reason of it is not clear, but it is presumed that the abrasive particles are not exposed from the surface in the binder and thus, cannot demonstrate the abrasive ability.

The process for producing the abrasive tape **10** is next explained.

First prepared is the base **11** for abrasive tape made of a polyester film, for example a biaxially oriented polyethylene terephthalate, and having the thickness of 10 to 200  $\mu\text{m}$ , preferably the thickness of 50 to 100  $\mu\text{m}$ . Next, the primer layer **12** mainly containing, for example, the epoxy resin, the acrylic resin, or the polyester resin is applied, if necessary, onto the abrasive tape **10**. This coating of the primer layer **12** prevents the abrasive layer **13** from being peeled off from the base **11** for abrasive tape while the optical fiber **2** is ground by the abrasive tape **10**.

The coating agent is next prepared by mixing the colloidal silica sol (abrasive particle solution) containing, for example, colloidal silica particles of the average particle size in the range of 1 to 200  $\mu\text{m}$  and the abrasive particle solvent such as isopropyl alcohol with the binder resin solution containing, for example, the organic-inorganic composite polymer resin (binder) and the binder solution such as isopropyl alcohol.

In this case, the colloidal silica particles maintain the average particle size in the range of 1 to 200  $\mu\text{m}$  in the coating agent, as being dispersed without cohesion.

A curing agent for curing the organic-inorganic composite polymer resin, for example an organic metal solution such as a tin compound, may be mixed in the coating agent, and a dispersing agent for dispersing the colloidal silica particles, for example a nonionic surfactant, may also be mixed in the coating agent.

In the case where the curing agent is mixed in the coating agent, a ratio of a solution of the curing agent to the organic-inorganic composite polymer resin (solid content) is preferably 90:10.

A P/V weight ratio, which is colloidal silica particles (solid content)/organic-inorganic composite polymer silicone resin (solid content), in the coating agent is in the range

of 20:80 to 95:5 (weight ratio), and preferably, the P/V weight ratio=50:50 to 80:20.

The coating agent is next applied by the gravure reverse process onto the primer layer **12** on the base **11** for abrasive tape. After the coating agent is applied onto the primer layer **12** on the base **11** for abrasive tape, the base **11** for abrasive tape is immediately heated at the temperature of 110°C. to 120°C. for 30 seconds, and during this period the solvent including isopropyl alcohol in the coating agent is scattered into the air.

Next, if the curing agent is mixed in the coating agent, the base **11** for abrasive tape is further heated at 80°C. for 10 minutes. On the contrary, if the curing agent is not mixed in the coating agent, the base **11** for abrasive tape is heated at 100°C. for one hour. The coating agent is thus dried to form the abrasive layer **13** in the thickness of 0.5 to 10  $\mu\text{m}$ , preferably 3 to 5  $\mu\text{m}$ , on the primer layer **12**, thus obtaining the abrasive tape **10**.

After the coating agent is dried under the above conditions, the colloidal silica particles can be dispersed as maintaining the average particle size in the range of 1 to 200  $\mu\text{m}$  in the abrasive layer **13** without cohesion.

Namely, unless the solvent including isopropyl alcohol is scattered immediately after application of the coating agent, the average particle size of the colloidal silica particles becomes large because the time is given for cohesion of the colloidal silica particles in the coating agent.

As described above, the colloidal silica particles in the coating agent can maintain the average particle size in the range of 1 to 200  $\mu\text{m}$  in all of the preparation step of the coating agent, the application step of the coating agent onto the primer layer **12**, and the drying step after that. Also, the colloidal silica particles maintain the average particle size in the range of 1 to 200  $\mu\text{m}$  in the abrasive layer **13**.

The reason why the colloidal silica particles maintain the average particle size in the range of 1 to 200  $\mu\text{m}$  is approximately as follows.

Generally, if the coating agent is prepared by dispersing particles of particle diameters of 1 or less  $\mu\text{m}$  in a binder resin solution such as a polyester, a polyester urethane, or a polyvinyl chloride-polyvinyl acetate copolymer, which is widely used as a binder resin solution, coarse particles of 5 to 10  $\mu\text{m}$  are likely to be made because of cohesion. Because of that, the abrasive tape having the abrasive layer formed using this coating agent forms scars on the ground body due to the coarse particles in the abrasive layer.

On the contrary, there are no such coarse particles of 5 to 10  $\mu\text{m}$  formed in the coating agent prepared by mixing the colloidal silica sol containing the colloidal silica particles of the average particle size in the range of 1 to 200  $\mu\text{m}$  with the binding resin solution containing the organic-inorganic composite polymer resin, according to the present invention. Because of that, the abrasive sheet having the abrasive layer formed using this coating agent becomes the abrasive sheet suitable for finishing of the end face of optical connector ferrule and the end face of semiconductor wafer **1**.

According to the present invention, the colloidal silica as the abrasive particles has the silanol group while the organic-inorganic composite polymer resin in the resin solution has a functional group such as polysiloxane oligomer having the framework of Si atoms. This polysiloxane oligomer is a functional group with high affinity to the silanol group, and, therefore, colloidal silica can be dispersed without cohesion in the binder resin solution. In the coating agent prepared by mixing the colloidal silica sol in which colloidal silica is stably dispersed in the organic solvent such as isopropyl alcohol, with the resin solution with low

viscosity similarly containing the organic solvent such as isopropyl alcohol, the colloidal silica sol and the binder resin solution contain the same or similar organic solvents, which facilitates dispersion of colloidal silica in the binder resin solution and which can suppress formation of aggregates of colloidal silica in the coating agent. These organic solvents may be selected from methanol, ethanol, xylene-butanol, ethylene glycol, ethylene glycol-mono n-propyl ether, dimethylacetamide, and methyl isobutyl ketone, as well as isopropyl alcohol.

If the base **11** for abrasive tape, the primer layer **12**, and the abrasive layer **13** in the abrasive tape **10** all have transparency, it is hard to distinguish the surface of the base from the surface of the abrasive layer, which could cause erroneous use. To prevent it, the base for abrasive tape may be subjected to coloring or printing of character or pattern.

Using the abrasive tape thus produced, the end face of optical connector ferrule or the surface of semiconductor wafer **1** is ground. Next explained is a method for grinding a surface of optical connector ferrule **2**.

As shown in FIG. 3, the abrasive tape **10** according to the present invention is placed through the elastic body **15** of elastomer on the rotating metal plate **16**, and the surface of optical connector ferrule **2** is ground with a lubricant of water for about two minutes on the abrasive tape **10**. Since the abrasive layer **13** of the abrasive tape **10** has no coarse particles of 5 to 10 $\mu$  due to cohesion as described above, the surface of optical connector ferrule **2** can be ground with efficiency.

Namely, the optical connector ferrule **2** can be ground uniformly and precisely by avoiding formation of the coarse particles of 5 to 10 $\mu$  due to cohesion in the abrasive layer **13** of the abrasive tape **10** as in the present invention. Since no scar is formed on the optical connector ferrule **2**, there is no need to supply an abrasive solution containing another abrasive during grinding. Some ground bodies can be further efficiently ground when a lubricant is supplied during grinding. The lubricant may be one generally known, such as water, alcohol, a surfactant, oil or the like. In this case, no abrasive is contained in the lubricant. When the lubricant is used, handling is easier and workability is better than in the mechanical polishing using an abrasive solution containing an abrasive.

During grinding, no clogging occurs in the abrasive layer **13** of the abrasive tape **10** and the abrasive layer **13** gradually decreases as a whole. Thus, since the life of the abrasive tape **10** continues as long as the abrasive layer **13** exists, the life of the abrasive tape **10** can be maintained long.

The same effect can be achieved when the precision component such as the semiconductor wafer **1** is ground instead of the optical connector ferrule **2**.

#### First Embodiment

The first embodiment of the present invention is next explained. The first embodiment corresponds to the first embodied form.

Specific examples of the abrasive tape and the production process thereof according to the present invention will be explained based on the following examples.

#### EXAMPLE 1

##### Coating agent for Abrasive Layer

10 parts by weight of a water-based silica sol [Snowtex 30 available from Nissan Chemical Industries] having the average particle size in the range of 10 to 20  $\mu$  was added to 10 parts by weight of a water-dispersed polymer polyester resin solution [Vylonal MD 1200 available from TOYOB CO., LTD.] and thereafter the mixture was stirred, thereby

obtaining the coating agent [a] for abrasive layer having the viscosity of 100 cps.

##### Production of Abrasive Tape

The above coating agent [a] for abrasive layer was applied in 20 g (dry)/m<sup>2</sup> by the three-roll reverse process on one side of the base for abrasive tape comprised of a polyethylene terephthalate film [low heat shrinkage SG type available from TEIJIN LTD.] having the thickness of 50 $\mu$ , and it was dried, thereby obtaining the abrasive tape (A) as an example product of the present invention.

This abrasive tape (A) was used to remove the haze as finishing of the surface of a 5-inch silicon wafer, which confirmed that finishing was able to be completed without any grinding scar or grinding spot.

#### EXAMPLE 2

##### Coating Agent for Abrasive Layer

A mixture solution of 10 parts by weight of the water-based silica sol [Snowtex 30 available from Nissan Chemical Industries] having the average particle size in the range of 10 to 20  $\mu$  with 10 parts by weight of the water-dispersed polymer polyester resin solution [Vylonal MD 1200 available from TOYOB CO., LTD.] was adjusted by an organic acid to pH 7.5, thereafter the mixture was stirred slowly for four hours, and then the mixture was filtered by a filter of 0.8 $\mu$ , thereby obtaining the coating agent [b] for abrasive layer having the viscosity of 100 cps.

##### Production of Abrasive Tape

The above coating agent [b] for abrasive layer was applied in 20 g (dry)/m<sup>2</sup> by the three-roll reverse process on one side of the base for abrasive tape comprised of the polyethylene terephthalate film [low heat shrinkage SG type available from TEIJIN LTD.] having the thickness of 50 $\mu$ , and it was dried, thereby obtaining the abrasive tape (B) as an example product of the present invention.

The abrasive layer in the abrasive tape (B) was whitened, from which it is apparent that aggregates of silica particles occurred in the abrasive layer.

The abrasive layer of the abrasive tape (B) was observed with an electron microscope, and it was confirmed that the particle diameters of the silica particles in the abrasive layer ranged from 0.1 to 0.8 $\mu$  (100 to 800  $\mu$ ).

This abrasive tape (B) was used to remove the haze as finishing of the surface of 5-inch silicon wafer, from which grinding performance of 0.1 $\mu$  or better was confirmed.

#### EXAMPLE 3

##### Coating Agent for Abrasive Layer

10 parts by weight of the isopropanol silica sol [IPA-ST available from Nissan Chemical Industries] having the average particle size in the range of 10 to 20  $\mu$  was added to 10 parts by weight of a silicone based coating agent [Glassca HPC 7502 available from Japan Synthetic Rubber], and thereafter the mixture was stirred, thereby obtaining the coating agent [c] for abrasive layer having the viscosity of 100 cps.

##### Production of Abrasive Tape

The above coating agent [c] for abrasive layer was applied in 20 g (dry)/m<sup>2</sup> by the three-roll reverse process on one side of the base for abrasive tape comprised of the polyethylene terephthalate film [low heat shrinkage SG type available from TEIJIN LTD.] having the thickness of 50 $\mu$ , and it was dried, thereby obtaining the abrasive tape (C) as an example product of the present invention.

This abrasive tape (C) was used to grind the end face of optical connector ferrule, which confirmed that finishing was able to be performed with little grinding scar or grinding spot.

## 11

## EXAMPLE 4

The coating agent [c] for abrasive layer used in Example 3 was applied in 30 g (dry)/m<sup>2</sup> by the three-roll reverse process onto one surface of the base for abrasive tape comprised of the polyethylene terephthalate film [low heat shrinkage SG type available from TEIJIN LTD.] having the thickness of 50 $\mu$  and thereafter the resultant was dried, thereby obtaining the abrasive tape (D) having the abrasive layer of the thickness 20 $\mu$  as an example product of the present invention.

When this abrasive tape (D) was used to grind the end face of optical connector ferrule, mirror finishing was achieved without any grinding scar or grinding spot, thereby obtaining the optical connector ferrule excellent in the damping property of signal.

## EXAMPLE 5

## Coating Agent for Abrasive Layer

The colloidal silica [Snowtex 30 available from Nissan Chemical Industries] having the average particle size in the range of 10 to 20 m $\mu$  was mixed at polyester resin/silica=1/1 (weight ratio) into a water-dispersed polyester resin solution [Vylonal MD-1245 available from TOYOB CO., LTD.] and thereafter an ammonia solution was added thereto to adjust it to pH 7.

After the mixture was stirred for two hours, it was filtered by the filter of 0.8 $\mu$  to obtain the coating agent [e] for abrasive layer.

## Production of Abrasive Tape

The above coating agent [e] for abrasive layer was applied in 30 g (dry)/m<sup>2</sup> by the three-roll reverse process on one side of the base for abrasive tape comprised of the polyethylene terephthalate film [low heat shrinkage SG type available from TEIJIN LTD.] having the thickness of 50 $\mu$ , and it was dried, thereby obtaining the abrasive tape (E) as an example product of the present invention.

When this abrasive tape (E) was used to grind the end face of optical connector ferrule, mirror finishing was achieved without any grinding scar or grinding spot, thereby obtaining the optical connector ferrule excellent in the damping property of signal.

## Second Embodiment

The second embodiment is next explained. The second embodiment corresponds to the second embodied form.

## EXAMPLE 6

## Coating Agent for Abrasive Layer

80 parts by weight of a colloidal silica sol [Organosilica sol IPA-ST, isopropyl alcohol solvent, solid content 30% available from Nissan Chemical Industries] having the average particle size in the range of 10 to 15 m $\mu$  was added to 20 parts by weight of an organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (f) for abrasive layer.

80 parts by weight of the colloidal silica sol [organosilica sol IPA-ST, isopropyl alcohol solvent, solid content 30% available from Nissan Chemical Industries] having the average particle size in the range of 10 to 15 m $\mu$  and 2 parts by weight of a curing agent [HPC 404H available from Japan Synthetic Rubber] were added to 20 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (g) for abrasive layer.

## 12

3 parts by weight of a dispersing agent [a carboxylic acid dispersing agent available from Japan Synthetic Rubber], 80 parts by weight of the colloidal silica sol [Organosilica sol IPA-ST, isopropyl alcohol solvent, solid content 30% available from Nissan Chemical Industries] having the average particle size in the range of 10 to 15 m $\mu$ , and 2 parts by weight of the curing agent [HPC 404H available from Japan Synthetic Rubber] were added to 20 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (h) for abrasive layer.

Here are the characteristics of the above materials, Glassca HPC 7502, HPC 404H, and IPA-ST shown in the following table.

TABLE 1

|    | Glassca HPC7502    | HPC4O4H               | IPA-ST                 |
|----|--------------------|-----------------------|------------------------|
| 20 | Solvent Methanol   | Solvent Isobutanol    | Solvent Isopropanol    |
|    | Solid content 31%  | Solid content         | Solid content          |
| 25 | Viscosity 4-16 cps | Less than 1% 2-15 cps | 30% Viscosity 3-20 cps |

## Process for Producing the Abrasive Tape

The above coating agent for abrasive layer (f), (g) or (h) was subjected to filtering at filtration accuracy of 1 $\mu$ . Then 30 the above coating agent (f), (g) or (h) was applied in 5 g (dry)/m<sup>2</sup> by the gravure reverse process (screen ruling plate of 95 rulings and plate depth 80 $\mu$ ) onto one surface (adhesion-enhanced surface) of the base for abrasive tape comprised of a polyethylene terephthalate film [adhesion-enhanced Melinex 542 type available from ICI Japan] having the thickness of 75 $\mu$  and the resultant was heated and dried, thereby obtaining the abrasive tape (F) (when the coating agent (f) for abrasive layer was used), (G) (when the coating agent (g) for abrasive layer was used), or (H) (when the coating agent (h) for abrasive layer was used) having the abrasive layer in the thickness of 3 $\mu$  (dry).

On the other hand, an anchor coating [an epoxy based anchor coating available from Japan Synthetic Rubber] was applied in 1 g (dry)/m<sup>2</sup> by the gravure reverse process 45 (screen ruling plate of 200 rulings and plate depth 30 $\mu$ ) onto one surface (corona-treated surface) of the base for abrasive tape comprised of a polyethylene terephthalate film [corona-treated E 5100 type available from TOYOB CO., LTD.] having the thickness of 75 $\mu$  to form the primer layer. Then 50 the above coating agent (f), (g) or (h) for abrasive layer was applied each in 5 g (dry)/m<sup>2</sup> by the gravure reverse process (screen ruling plate of 95 rulings and plate depth of 80 $\mu$ ) onto the primer layer and the resultant was heated and dried, thereby obtaining the abrasive tape F' (when the coating agent (f) for abrasive layer was used), G' (when the coating agent (g) for abrasive layer was used), or H' (when the coating agent (h) for abrasive layer was used) having the abrasive layer in the thickness of 3 $\mu$  (dry).

The abrasive layer in each abrasive tape (F), (G), (H), (F'), 60 (G'), (H') obtained by the above process did not contain the coarse particles of 5 to 10 $\mu$  due to cohesion of abrasive particles, and the arithmetical mean deviation (Ra) of the surface of the abrasive layer was as fine as about 0.1 $\mu$ . Here, the arithmetical mean deviation (Ra) of the surface of each 65 abrasive layer was measured by the surface roughness configuration meter, Surfcom 590A available from TOKYO SEIMITSU, with the cut-off value 0.8 mm (the same mea-

## 13

surement was carried out also in below Examples 7 to 13). The total ray transmittance of the abrasive tape (F) was 91% and the haze thereof was 9%, showing transparency.

## EXAMPLE 7

## Coating Agent for Abrasive Layer

70 parts by weight of the colloidal silica sol [Organosilica sol IPA-ST, isopropyl alcohol solvent, solid content 30% available from Nissan Chemical Industries] having the average particle size in the range of 10 to 15  $\mu$  was added to 30 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (i) for abrasive layer.

## Process for Producing the Abrasive Tape

The above coating agent for abrasive layer (i) was subjected to filtering at filtration accuracy of  $1\mu$ . Then the above coating agent (i) was applied in 5 g (dry)/ $m^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (I) having the abrasive layer in the thickness of  $3\mu$  (dry).

The abrasive layer in the abrasive tape (I) obtained by the above process did not contain the coarse particles of 5 to  $10\mu$  due to cohesion of abrasive particles, and the arithmetical mean deviation (Ra) of the surface of the abrasive layer was as fine as about  $0.2\mu$ . The total ray transmittance of the abrasive tape was 92% and the haze was 10%, thus showing transparency.

## EXAMPLE 8

## Coating Agent for Abrasive Layer

65 parts by weight of the colloidal silica sol [Organosilica sol IPA-ST, isopropyl alcohol solvent, solid content 30% available from Nissan Chemical Industries] having the average particle size in the range of 10 to 15  $\mu$  was added to 35 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (j) for abrasive layer.

## Process for Producing the Abrasive Tape

The above coating agent for abrasive layer (j) was subjected to filtering at filtration accuracy of  $1\mu$ . Then the above coating agent (j) was applied in 5 g (dry)/ $m^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (J) having the abrasive layer in the thickness of  $3\mu$  (dry).

The abrasive layer in the abrasive tape (J) obtained by the above process did not contain the coarse particles of 5 to  $10\mu$  due to cohesion of abrasive particles, and the arithmetical mean deviation (Ra) of the surface of the abrasive layer was as fine as about  $0.1\mu$ . The total ray transmittance of the abrasive tape was 92% and the haze was 13%, thus showing transparency.

## 14

## EXAMPLE 9

## Coating Agent for Abrasive Layer

200 parts by weight of the colloidal silica sol [Organosilica sol IPA-ST, isopropyl alcohol solvent, solid content 30% available from Nissan Chemical Industries] having the average particle size in the range of 10 to 15  $\mu$  was added to 30 parts by weight of a silicone varnish [KR-220IPA, isopropyl alcohol solvent, solid content 51% available from Shin-Etsu Kagaku Kogyo] and thereafter 10 ultrasonic dispersion was carried out, thereby obtaining the coating agent (k) for abrasive layer.

## Process for Producing the Abrasive Tape

The above coating agent for abrasive layer (k) was subjected to filtering at filtration accuracy of  $1\mu$ . Then the above coating agent (k) was applied in 5 g (dry)/ $m^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (K) having the abrasive layer in the thickness of  $3\mu$  (dry).

The abrasive layer in the abrasive tape (K) obtained by the above process did not contain the coarse particles of 5 to  $10\mu$  due to cohesion of abrasive particles, and the arithmetical mean deviation (Ra) of the surface of the abrasive layer was as fine as 0.3 or less  $\mu$ . The abrasive tape had transparency.

## EXAMPLE 10

## Coating Agent for Abrasive Layer

80 parts by weight of the colloidal silica sol [Organosilica sol IPA-ST, isopropyl alcohol solvent, solid content 30% available from Nissan Chemical Industries] having the average particle size in the range of 70 to 100  $\mu$  was added to 20 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (l) for abrasive layer.

## Process for Producing the Abrasive Tape

The above coating agent for abrasive layer (l) was subjected to filtering at filtration accuracy of  $1\mu$ . Then the above coating agent (l) was applied in 5 g (dry)/ $m^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (L) having the abrasive layer in the thickness of  $3\mu$  (dry).

The abrasive layer in the abrasive tape (L) obtained by the above process did not contain the coarse particles of 5 to  $10\mu$  due to cohesion of abrasive particles, and the arithmetical mean deviation (Ra) of the surface of the abrasive layer was as fine as about  $0.2\mu$ . The total ray transmittance of the abrasive tape was 85% and the haze was 61%, thus showing semitransparency.

## EXAMPLE 11

## Coating Agent for Abrasive Layer

70 parts by weight of the colloidal silica sol [Organosilica sol IPA-ST, isopropyl alcohol solvent, solid content 30% available from Nissan Chemical Industries] having the average particle size in the range of 70 to 100  $\mu$  was added to 30 parts by weight of the organic-inorganic composite

## 15

polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (m) for abrasive layer.

## Process for Producing the Abrasive Tape

The above coating agent for abrasive layer (m) was subjected to filtering at filtration accuracy of  $1\mu$ . Then the above coating agent (m) was applied in  $5\text{ g (dry)}/\text{m}^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (M) having the abrasive layer in the thickness of  $3\mu$  (dry).

The abrasive layer in the abrasive tape (M) obtained by the above process did not contain the coarse particles of 5 to  $10\mu$  due to cohesion of abrasive particles, and the arithmetical mean deviation (Ra) of the surface of the abrasive layer was as fine as about  $0.2\mu$ . The total ray transmittance of the abrasive tape was 87% and the haze was 68%, thus showing semitransparency.

## EXAMPLE 12

## Coating Agent for Abrasive Layer

60 parts by weight of the colloidal silica sol [Organosilica sol IPA-ST, isopropyl alcohol solvent, solid content 30% available from Nissan Chemical Industries] having the average particle size in the range of 70 to 100  $\text{m}\mu$  was added to 40 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (n) for abrasive layer.

## Process for Producing the Abrasive Tape

The above coating agent for abrasive layer (n) was subjected to filtering at filtration accuracy of  $1\mu$ . Then the

5

## 16

mean deviation (Ra) of the surface of the abrasive layer was as fine as about  $0.2\mu$ . The total ray transmittance of the abrasive tape was 89% and the haze was 46%, thus showing semitransparency.

## EXAMPLE 13

## Coating Agent for Abrasive Layer

50 parts by weight of the colloidal silica sol [Organosilica sol IPA-ST, isopropyl alcohol solvent, solid content 30% available from Nissan Chemical Industries] having the average particle size in the range of 70 to 100  $\text{m}\mu$  was added to 50 parts by weight of the organic-inorganic composite polymer silicone resin solution [ceramic coat material Glassca HPC 7502, methanol solvent, solid content 30% available from Japan Synthetic Rubber] and thereafter ultrasonic dispersion was carried out, thereby obtaining the coating agent (o) for abrasive layer.

## Process for Producing the Abrasive Tape

The above coating agent for abrasive layer (o) was subjected to filtering at filtration accuracy of  $1\mu$ . Then the above coating agent (o) was applied in  $5\text{ g (dry)}/\text{m}^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (O) having the abrasive layer in the thickness of  $3\mu$  (dry).

The abrasive layer in the abrasive tape (O) obtained by the above process did not contain the coarse particles of 5 to  $10\mu$  due to cohesion of abrasive particles, and the arithmetical mean deviation (Ra) of the surface of the abrasive layer was as fine as about  $0.2\mu$ . The total ray transmittance of the abrasive tape was 90% and the haze was 20%, thus showing transparency.

Table 2 below shows results of evaluation about the total ray transmittance, haze, appearance, and grinding characteristics of optical connector for the abrasive tapes (F), (I), (J), (L), (M), (N), (O) obtained by the above processes.

TABLE 2

| Abrasive tape | Silica average particle size ( $\text{m}\mu$ ) | PV ratio silica/binder (weight ratio) | Total ray transmittance (%) | Haze (%) | Appearance | Grinding characteristics of optical connector |
|---------------|------------------------------------------------|---------------------------------------|-----------------------------|----------|------------|-----------------------------------------------|
| Example 6     | F                                              | 10-15                                 | 80/20                       | 91       | 9          | Transparent                                   |
| Example 7     | I                                              | 10-15                                 | 70/30                       | 92       | 10         | Transparent                                   |
| Example 8     | J                                              | 10-15                                 | 65/35                       | 92       | 13         | Transparent                                   |
| Example 10    | L                                              | 70-100                                | 80/20                       | 85       | 61         | Semitransparent                               |
| Example 11    | M                                              | 70-100                                | 70/30                       | 87       | 68         | Semitransparent                               |
| Example 12    | N                                              | 70-100                                | 60/40                       | 89       | 46         | Semitransparent                               |
| Example 13    | O                                              | 70-100                                | 50/50                       | 90       | 20         | Transparent                                   |

above coating agent (n) was applied in  $5\text{ g (dry)}/\text{m}^2$  by the gravure reverse process (screen ruling plate of 95 rulings and plate depth  $80\mu$ ) onto one surface (adhesion-enhanced surface) of the base for abrasive tape comprised of the polyethylene terephthalate film [adhesion-enhanced Melinex 542 type available from ICI Japan] having the thickness of  $75\mu$  and the resultant was heated and dried, thereby obtaining the abrasive tape (N) having the abrasive layer in the thickness of  $3\mu$  (dry).

The abrasive layer in the abrasive tape (N) obtained by the above process did not contain the coarse particles of 5 to  $10\mu$  due to cohesion of abrasive particles, and the arithmetical

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
5510  
5511  
5512  
5513  
5514  
5515  
5516  
5517  
5518  
5519  
5520  
5521  
5522  
5523  
5524  
5525  
5526  
5527  
5528  
5529  
5530  
5531  
5532  
5533  
5534  
5535  
5536  
5537  
5538  
5539  
55310  
55311  
55312  
55313  
55314  
55315  
55316  
55317  
55318  
55319  
55320  
55321  
55322  
55323  
55324  
55325  
55326  
55327  
55328  
55329  
55330  
55331  
55332  
55333  
55334  
55335  
55336  
55337  
55338  
55339  
55340  
55341  
55342  
55343  
55344  
55345  
55346  
55347  
55348  
55349  
55350  
55351  
55352  
55353  
55354  
55355  
55356  
55357  
55358  
55359  
55360  
55361  
55362  
55363  
55364  
55365  
55366  
55367  
55368  
55369  
55370  
55371  
55372  
55373  
55374  
55375  
55376  
55377  
55378  
55379  
55380  
55381  
55382  
55383  
55384  
55385  
55386  
55387  
55388  
55389  
55390  
55391  
55392  
55393  
55394  
55395  
55396  
55397  
55398  
55399  
553100  
553101  
553102  
553103  
553104  
553105  
553106  
553107  
553108  
553109  
553110  
553111  
553112  
553113  
553114  
553115  
553116  
553117  
553118  
553119  
553120  
553121  
553122  
553123  
553124  
553125  
553126  
553127  
553128  
553129  
553130  
553131  
553132  
553133  
553134  
553135  
553136  
553137  
553138  
553139  
553140  
553141  
553142  
553143  
553144  
553145  
553146  
553147  
553148  
553149  
553150  
553151  
553152  
553153  
553154  
553155  
553156  
553157  
553158  
553159  
553160  
553161  
553162  
553163  
553164  
553165  
553166  
553167  
553168  
553169  
553170  
553171  
553172  
553173  
553174  
553175  
553176  
553177  
553178  
553179  
553180  
553181  
553182  
553183  
553184  
553185  
553186  
553187  
553188  
553189  
553190  
553191  
553192  
553193  
553194  
553195  
553196  
553197  
553198  
553199  
553200  
553201  
553202  
553203  
553204  
553205  
553206  
553207  
553208  
553209  
553210  
553211  
553212  
553213  
553214  
553215  
553216  
553217  
553218  
553219  
553220  
553221  
553222  
553223  
553224  
553225  
553226  
553227  
553228  
553229  
553230  
553231  
553232  
553233  
553234  
553235  
553236  
553237  
553238  
553239  
553240  
553241  
553242  
553243  
553244  
553245  
553246  
553247  
553248  
553249  
553250  
553251  
553252  
553253  
553254  
553255  
553256  
553257  
553258  
553259  
553260  
553261  
553262  
553263  
553264  
553265  
553266  
553267  
553268  
553269  
553270  
553271  
553272  
553273  
553274  
553275  
553276  
553277  
553278  
553279  
553280  
553281  
553282  
553283  
553284  
553285  
553286  
553287  
553288  
553289  
553290  
553291  
553292  
553293  
553294  
553295  
553296  
553297  
553298  
553299  
553300  
553301  
553302  
553303  
553304  
553305  
553306  
553307  
553308  
553309  
553310  
553311  
553312  
553313  
553314  
553315  
553316  
553317  
553318  
553319  
553320  
553321  
553322  
553323  
553324  
553325  
553326  
553327  
553328  
553329  
553330  
553331  
553332  
553333  
553334  
553335  
553336  
553337  
553338  
553339  
553340  
553341  
553342  
553343  
553344  
553345  
553346  
553347  
553348  
553349  
553350  
553351  
553352  
553353  
553354  
553355  
553356  
553357  
553358  
553359  
553360  
553361  
553362  
553363  
553364  
553365  
553366  
553367  
553368  
553369  
553370  
553371  
553372  
553373  
553374  
553375  
553376  
553377  
553378  
553379  
553380  
553381  
553382  
553383  
553384  
553385  
553386  
553387  
553388  
553389  
553390  
553391  
553392  
553393  
553394  
553395  
553396  
553397  
553398  
553399  
553400  
553401  
553402  
553403  
553404  
553405  
553406  
553407  
553408  
553409  
553410  
553411  
553412  
553413  
553414  
553415  
553416  
553417  
553418  
553419  
553420  
553421  
553422  
553423  
553424  
553425  
553426  
553427  
553428  
553429  
553430  
553431  
553432  
553433  
553434  
553435  
553436  
553437  
553438  
553439  
553440  
553441  
553442  
553443  
553444  
553445  
553446  
553447  
553448  
553449  
553450  
553451  
553452  
553453  
553454  
553455  
553456  
553457  
553458  
553459  
553460  
553461  
553462  
553463  
553464  
553465  
553466  
553467  
553468  
553469  
553470  
553471  
553472  
553473  
553474  
553475  
553476  
553477  
553478  
553479  
553480  
553481  
553482  
553483  
553484  
553485  
553486  
553487  
553488  
553489  
553490  
553491  
553492  
553493  
553494  
553495  
553496  
553497  
553498  
553499  
553500  
553501  
553502  
553503  
553504  
553505  
553506  
553507  
553508  
553509  
553510  
553511  
553512  
553513  
553514  
553515  
553516  
553517  
553518  
553519  
553520  
553521  
553522  
553523  
553524  
553525  
553526  
553527  
553528  
553529  
553530  
553531  
553532  
553533  
553534  
553535  
553536  
553537  
553538  
553539  
553540  
553541  
553542  
553543  
553544  
553545  
553546  
553547  
553548  
553549  
553550  
553551  
553552  
553553  
553554  
553555  
553556  
553557  
553558  
553559  
553560  
553561  
553562  
553563  
553564  
553565  
553566  
553567  
553568  
553569  
553570  
553571  
553572  
553573  
553574  
553575  
553576  
553577  
553578  
553579  
553580  
553581  
553582  
553583  
553584  
553585  
553586  
553587  
553588  
553589  
553590  
553591  
553592  
553593  
553594  
553595  
553596  
553597  
553598  
553599  
553600  
553601  
553602  
553603  
553604  
553605  
553606  
553607  
553608  
553609  
553610  
553611  
553612  
553613  
553614  
553615  
553616  
553617  
553618  
553619  
553620  
553621  
553622  
553623  
553624  
553625  
553626  
553627  
553628  
553629  
553630  
553631  
553632  
553633  
553634  
553635  
553636  
553637  
553638  
553639  
553640  
553641  
553642  
553643  
553644  
553645  
553646  
553647  
553648  
553649  
553650  
553651  
553652  
553653  
553654  
553655  
553656  
553657  
553658  
553659  
553660  
553661  
553662  
553663  
553664  
553665  
553666  
553667  
553668  
553669  
553670  
553671  
553672  
553673  
553674  
553675  
553676  
553677  
553678  
553679  
553680  
553681  
553682  
553683  
553684  
553685  
553686  
553687  
553688  
553689  
553690  
553691  
553692  
553693  
553694  
553695  
553696  
553697  
553698  
553699  
553700  
553701  
553702  
553703  
553704  
553705  
553706  
553707  
553708  
553709  
553710  
553711  
553712  
553713  
553714  
553715  
553716  
553717  
553718  
553719  
553720  
553721  
553722  
553723  
553724  
553725  
553726  
553727  
553728  
553729  
553730  
553731  
553732  
553733  
553734  
553735  
553736  
553737  
553738  
553739  
5537340  
5537341  
5537342  
5537343  
5537344  
5537345  
5537346  
5537347  
5537348  
5537349  
5537350  
5537351  
553735

three-dimensional surface roughness configuration analysis system, Surfcom 590A-3DF available from TOKYO SEIMITSU.

#### COMPARATIVE EXAMPLE 1

200 parts by weight of aluminum oxide fine powder [WA#10000 available from Showa Denko K. K.] having the average particle size 800  $\mu$ m was added into a resin solution containing 50 parts by weight of a linear saturated polyester resin [Vylon #530 available from TOYOB CO., LTD.], 70 parts by weight of toluene, and 70 parts by weight of methyl ethyl ketone, the mixture was well dispersed by sand mill, and thereafter it was diluted with an equal-amount mixture solvent of toluene and methyl ethyl ketone, thereby obtaining the coating agent [p] for abrasive layer having the viscosity of 100 cps.

The above coating agent [p] for abrasive layer was applied in 40 g (dry)/ $m^2$  by the three-roll reverse process onto one surface (corona-treated surface) of the base for abrasive tape comprised of the polyethylene terephthalate film [corona-treated E 5100 type available from TOYOB CO., LTD.] having the thickness of 75 $\mu$  and thereafter the resultant was heated and dried, thereby obtaining the abrasive tape (P) as a product of a comparative example.

#### COMPARATIVE EXAMPLE 2

400 parts by weight of the colloidal silica sol [Organosilica sol MEK-ST, methyl ethyl ketone solvent, solid content 30% available from Nissan Chemical Industries] containing colloidal silica having the average particle size in the range of 10 to 20  $\mu$ m was added into a resin solution containing 30 parts by weight of the linear saturated polyester resin [Vylon #530 available from TOYOB CO., LTD.], 40 parts by weight of toluene, and 40 parts by weight of methyl ethyl ketone and thereafter it was diluted with the equal-amount mixture solvent of toluene and methyl ethyl ketone, thereby obtaining the coating agent [q] for abrasive layer having the viscosity of 20 cps.

The above coating agent [q] for abrasive layer was applied in 5 g (dry)/ $m^2$  by the gravure reverse process (screen ruling plate of 95 rulings and plate depth of 80 $\mu$ ) onto one surface (corona-treated surface) of the base for abrasive tape comprised of the polyethylene terephthalate film [corona-treated E 5100 type available from TOYOB CO., LTD.] having the thickness of 75 $\mu$  and thereafter the resultant was heated and dried, thereby obtaining the abrasive tape (Q) as a product of a comparative example.

Finishing of the end face of optical connector ferrule was carried out using the abrasive tapes (P) and (Q) obtained in Comparative Examples 1, 2, and the results showed that there were grinding scars and grinding spots on the surface of the end face of ferrule and the grinding characteristics thereof were not good.

Neither of the abrasive layers of the abrasive tapes (F), (G), (H), (F'), (G'), (H'), (I), (J), (K), (L), (M), (N), and (O) obtained by the above processes contains the coarse particles of 5 to 10 $\mu$  due to cohesion of abrasive particles, and the arithmetical mean deviation (Ra) of the surface of each abrasive layer was 0.3 or less  $\mu$ .

All the abrasive tapes of the above examples had good grinding characteristics of the end face of optical connector ferrule as compared with the abrasive tapes (P) and (Q) of the comparative examples, though they had transparency or, cloudy white or semitransparency depending upon the particle diameters of abrasive particles used or the formulation

rate of the abrasive particles and binder. Namely, when they were used for finishing of the end face of optical connector ferrule, mirror finishing was achieved without any grinding scar or grinding spot, thus obtaining the optical connector ferrule excellent in the damping characteristics of optical signal.

The same finishing grinding tests were carried out for precision components including semiconductor wafers, metals, ceramics, color filters (for liquid crystal display or the like), plasma displays, optical lenses, magnetic disk or optical disk substrates, magnetic heads, and optical reading heads, instead of the optical connector ferrule. As a result, the same results were achieved as in the case of the optical connector ferrule.

According to the present invention, because the abrasive particles in the abrasive layer are fine particles having small and close particle diameters and there are no coarse particles of 5 to 10 $\mu$  in the abrasive layer, finishing can be performed without grinding scar or grinding spot on the surface or the like of the precision component such as the optical connector ferrule or the semiconductor wafer.

Furthermore, the abrasive tape suitable for finishing and high in grinding performance can be obtained easily and certainly.

Furthermore, because the average particle size of the abrasive particles in the abrasive layer is maintained in the range of 1 to 200  $\mu$ m, the precision component such as the optical connector ferrule or the semiconductor wafer can be ground without any scar on the surface.

Furthermore, the coating agent can be obtained containing the abrasive having the average particle size in the range of 1 to 200  $\mu$ m.

Furthermore, the abrasive tape suitable for finishing can be obtained easily and certainly.

What is claimed is:

1. An abrasive tape comprising:

a base; and

an abrasive layer formed on the base;

wherein the abrasive layer is formed from a coating agent in which colloidal silica particles of an average particle size in the range of 10 to 100  $\mu$ m of a colloidal silica sol are dispersed in a binder resin solution.

2. The abrasive tape according to claim 1, wherein said binder resin solution has a silicone resin or a silicone based resin.

3. The abrasive tape according to claim 1, wherein particle diameters of the abrasive particles in the abrasive layer are between 50 and 800  $\mu$ m.

4. An abrasive tape comprising:

a base; and

an abrasive layer formed on the base;

wherein said abrasive layer has colloidal silica particles of an average particle size in the range of 1 to 200  $\mu$ m of a colloidal silica sol and a binder for binding the abrasive particles.

5. The abrasive tape according to claim 4, wherein said binder is a binder having siloxane bonding.

6. The abrasive tape according to claim 4, wherein a total ray transmittance of the abrasive layer is 60 to 95% and a haze thereof is 1 to 70%.

7. The abrasive tape according to claim 4, wherein a primer layer is provided between the base for abrasive tape and the abrasive layer.